

## UNITED STATES PATENT OFFICE

2,040,796

PROCESS OF DYEING ANIMAL FIBERS WITH  
METAL COMPLEX COMPOUNDS OF OR-  
GANIC ACID DYESTUFFSCarl Maria Rittinghausen, Bad Soden-on-the-  
Taunus, and Richard Haynn, Frankfort-on-  
the-Main, Germany, assignors to General Ani-  
line Works, Inc., New York, N. Y., a corporation  
of DelawareNo Drawing. Application November 29, 1932,  
Serial No. 644,914. In Germany December 7,  
1931

9 Claims. (Cl. 8—5)

Our present invention relates to an improvement in the dyeing of animal fibers with metal complex compounds of organic acid dyestuffs, such as copper or chromium complex compounds of acid ortho-hydroxy-azo dyestuffs or other acid dyestuffs capable of forming metal complex compounds; more particularly it relates to a process which comprises carrying out the dyeing process in an acid bath containing only such a quantity of acid as is usual for dyeing with ordinary acid dyestuffs and in the presence of a water-soluble protective colloid of the group consisting of protective colloids of natural and synthetic origin.

It is known that in the dyeing process by means of metal complex compounds of acid organic dyestuffs, sulfuric acid or an organic acid together with sulfuric acid is added to the dye bath. In order to obtain a satisfactory evenness of the dyeings and a normal development of the fastness properties of the dyestuffs, the hitherto known process of dyeing with this class of dyestuffs requires a considerably high quantity of acid, for instance, about 8 to 10 per cent of sulfuric acid calculated on the weight of the material to be dyed, and prolonged boiling is required to finish the dyeing operation.

This method has the disadvantage that the dye baths are only insufficiently utilized, even when a high percentage of dyestuff is used, that the dye tubs or vessels are soon corroded and that the vegetable effect threads contained in the woolen or other animal materials are injured. The use of formic acid or of formic acid together with sulfuric acid, as suggested in the French Patent No. 702,387 yields, in the case of most of the metal complex compounds of acid dyestuffs, mixture (uneven and spotted) dyeings which, with the exception of a few cases, do not possess the normal and characteristic fastness properties of the dyestuffs proper. Furthermore, this latter method is not suited for the production of fancy (light) shades.

We have now found that the dyeing with metal complex compounds of organic acid dyestuffs, such as copper or chromium or other metal complex compounds of acid ortho-hydroxy azo dyestuffs or other acid dyestuffs capable of forming metal complex compounds, may be carried out in normal acid dye baths containing only the normal quantities of acid as are usual for dyeing with ordinary acid dyestuffs which do not contain metal in a complex binding, that is to say, with smaller quantities of sulfuric acid than those hitherto used for dyeing with the said class of

metal complex compounds of acid dyestuffs, if the dyeing operation is carried out in the presence of a water-soluble protective colloid of the group consisting of protective colloids of natural and synthetic origin. In the new process about 3 to at most 5 per cent, generally about 4 per cent, of sulfuric acid are sufficient.

The term "protective colloid" and the class of materials identified thereby and their properties are well known to those skilled in the art. There may be used in our present process all kinds of protective colloids, i. e. natural products, or products made from natural materials, or protective colloids made by synthesis. Furthermore, the process of the present invention is not limited to any particular class of metal complex compounds of acid dyestuffs; the effect obtained is evident in the case of all dyes included in the general meaning of the term "metal complex compounds of acid organic dyestuffs".

As water-soluble natural protective colloids or as protective colloids made from natural products there may be mentioned glue, starch, dextrin, derivatives of sugar, sulfite pulp waste liquors, water-soluble albuminous substances or decomposition products thereof, for instance, compounds of the kind of the so-called protalbinic- and lysalbinic acids, such as the mixture of the sodium salts of caseoprotalbinic- and caseolysalbinic acid obtainable by causing caustic soda to act upon casein. Compounds of this class are, for instance, disclosed by Paal in "Berichte der deutschen Chemischen Gesellschaft", volume 35, page 2195 and following.

Synthetic compounds which have the properties of protective colloids are, for instance, the compounds obtainable by introducing into organic compounds containing one or more hydroxy, carboxy or amino groups a radical of a polyglycol ether containing 4 or more  $C_2H_4$  groups, such as the radical—



and further combining, if desired, the thus obtained condensation products which still contain free hydroxyl groups with reactive compounds. Compounds of this kind are more fully disclosed in French Patent No. 727,202 and British Patents Nos. 380,431 and 380,851.

By these additions the efficiency of the dye baths is increased and very even dyeings are obtained; simultaneously the other disadvantages which appear if the old process with the high percentage of acid is used, are avoided. It is surprising that the addition of only a small quan-

tity of a water-soluble protective colloid allows the dyeing of animal fibers by means of metal complex compounds of acid dyestuffs in the presence of much less sulfuric acid and yet with better results than by the old method.

5 A further increase of the qualities of the dyeings may be attained if, in addition to the protective colloid, water-soluble salts of hydrohalic acids or similarly acting acids, such as chlorides, bromides, fluorides or thiocyanates, are added to the dye baths.

10 Accordance to our new process the dyeing operation in the presence of a water-soluble protective colloid may be carried out while using as an acid sulfuric acid, or sulfuric acid together with an organic acid, such as formic acid, or even an organic acid alone.

15 The following examples serve to illustrate the invention, but they are not intended to limit it thereto, the parts being by weight, unless stated otherwise: The percentage quantities are calculated on the weight of the material to be dyed:

(1) Wool is dyed as follows:

20 A dye bath is prepared from 6 per cent of the chromium complex compound of the diphenyl-naphthylmethane dyestuff from 1 mol. of 2-hydroxy-1-naphthaldehyde-3,6-disulfonic acid and 2 mols of ortho-cresotinic acid (obtainable by heating in an autoclave at 120° C. for 1 hour 100 parts of the dyestuff with 400 parts of a chromium formiate solution containing 5 per cent of Cr<sub>2</sub>O<sub>3</sub>), 4 per cent of sulfuric acid and 5 to 10 per cent of glue, the material is introduced into the dye bath, the whole is heated to boiling within half an hour and boiling is continued for 1 to 1½ hours.

25 (2) The dye bath is prepared from 6 per cent of the dyestuff used in Example (1), 4 per cent of sulfuric acid, 5 to 10 per cent of glue and 2½ per cent of ammonium fluoride or ammonium chloride and the material is treated as indicated in Example (1).

30 (3) Wool is dyed in a dye bath containing 6 per cent of the dyestuff used in Example (1), 4 per cent of formic acid of 85 per cent strength and 5 to 10 per cent of glue. The material is entered into the dye bath, the whole is heated to boiling temperature and the material is dyed at this temperature for 1 to 1½ hours.

35 50 Instead of glue there may be used the corresponding quantity of an albuminous decomposition product which is obtainable from casein by the action of caustic soda in the heat.

40 (4) The dye bath is prepared from 6 per cent of the chromium complex compound of the azo dyestuff from diazotized 1-amino-2-naphthol-4-sulfonic acid and β-naphthol (obtainable by heating in an autoclave at 105° C for 2 hours 100 parts of the azo dyestuff with 60 parts of a chromium salt and 1000 parts of water), 4 per cent of formic acid of 85 per cent strength and 5 to 10 per cent of glue or the same quantity of a water-soluble albuminous decomposition product. The material to be dyed is introduced into the dye bath, the whole is heated to boiling within ½ hour, the material is dyed at this temperature for ½ hour, 4 per cent of sulfuric acid of 96 per cent strength are added and boiling is continued for 1 hour.

45 50 (5) Wool is dyed as follows:

55 There is prepared a dye bath containing 6 per cent of the dyestuff used in Example (1), 4 per cent of sulfuric acid of 96 per cent strength and 2 to 3 per cent of a reaction product from ethylene oxide and dodecylalcohol, obtainable, for in-

stance, by heating 200 parts of dodecylalcohol to about 180° C. in an autoclave with about 400 parts of ethylene oxide which is introduced a little at a time. The material is introduced into the dye bath, the whole is heated to boiling within ½ hour and boiling is continued for 1 to 1½ hours.

60 (6) The dye bath is prepared from 6 per cent of the dyestuff used in Example (1), 4 per cent of sulfuric acid of 96 per cent strength, 2 to 3 per cent of a condensation product obtainable according to one of the examples of the British Specifications Nos. 380,431 and 380,851 or of the French Patent No. 727,202, for instance, a condensation product of 20 mols of ethylene oxide with 1 mol. of octodecylalcohol, obtainable by 10 leading about 880 parts of ethylene oxide, while stirring at a temperature between 130° C. and 140° C. into 270 parts of octodecylalcohol containing 2.7 parts of an aqueous caustic soda solution of 40° Bé., and 2.5 per cent of ammonium 15 fluoride or ammonium chloride. The material is dyed as indicated in Example 5.

15 (7) A dye bath is prepared from 6 per cent of the chromium complex compound of the dyestuff from diazotized 4-nitro-2-aminophenyl and 20 phenyl-2-amino-8-naphthol-6-sulfonic acid, 4 per cent of formic acid of 85 per cent strength and 2 to 3 per cent of the reaction product from ethylene oxide with dodecylalcohol mentioned in Example (5). Wool is dyed in this bath with or 25 without addition of ammonium fluoride or ammonium chloride.

20 (8) Wool is dyed in a bath which is prepared from 6 per cent of the dyestuff used in Example 1, 4 per cent of formic acid of 85 per cent strength, 30 2 to 3 per cent of the reaction product from ethylene oxide and dodecylalcohol. The whole is heated to boiling within ½ hour, the material is dyed at boiling temperature for ½ hour, 4 per cent of sulfuric acid of 96 per cent strength 35 are added and boiling is continued for 1 hour.

30 (9) A dye bath is prepared containing 4 per cent of a chromium complex compound of the azo dyestuff from diazotized nitro-1-amino-2-hydroxynaphthalene-4-sulfonic acid and β-naphthol, 4 per cent of sulfuric acid of 96 per cent strength and about 2 per cent of a poly-oxyethyl-ether of sorbit-tetra-palm oil fatty acid ester, obtainable by introducing ethylene oxide at 45 about 140° C. to about 160° C. and in the presence of 0.5 per cent of caustic soda solution of 40° Bé. into a melt of the sorbit-tetra-palm oil fatty acid ester, until about 70 mols of ethylene oxide per mol. of the ester have been absorbed. Sorbit-tetra-palm oil fatty acid ester is obtainable by 50 heating sorbit with a quantity of palm oil fatty acid necessary for forming the tetra-ester at about 200° C. to about 215° C. until free fatty acid is no longer detectable.

55 The dyeing operation is commenced at 40° C. 60 the material to be dyed is heated to boiling within ½ hour and boiling is continued for about 1 hour.

Instead of the protective colloids, used in the foregoing examples, the following compounds 65 may be used:

(a) 2 to 3 per cent. of a polyglycoether of wool fat alcohols;

(b) 2 to 3 per cent. of a product obtainable by condensation of oleylalcohol with 20 mols of 70 ethylene oxide and subsequent ethylation;

(c) 2 to 3 per cent. of a polyglycoether of ricinoleic acid (obtainable as described in Example 2 of British Patent No. 380,431);

(d) 2 to 3 per cent. of a product consisting of 75

95 parts of a condensation product, obtainable from oleic acid and 6 mols of ethylene oxide and subsequent ethylation, and 5 parts of product b).

We claim:

5 1. The process of dyeing animal fibers with metal complex compounds of organic acid dyestuffs which comprises carrying out the dyeing in normal acid dye baths, containing about 3 to 5 per cent of acid as is usual for dyeing with 10 ordinary acid dyestuffs, and in the presence of a water-soluble protective colloid.

15 2. A modification of the process as claimed in claim 1 which comprises adding to the dye bath a small quantity of a salt of the group consisting 15 of water-soluble salts of hydrohalic acids and thiocyanic acid.

20 3. The process of dyeing animal fibers with a metal complex compound of an organic acid dyestuff which comprises carrying out the dyeing in a normal acid dye bath containing about 4 per cent of sulfuric acid and about 2 to 10 per cent of a water-soluble protective colloid, calculated on the weight of the material to be dyed.

25 4. A modification of the process as claimed in claim 3 which comprises replacing the sulfuric acid by a corresponding quantity of formic acid.

30 5. The process of dyeing wool with a chromium complex compound of an organic acid dyestuff which comprises carrying out the dyeing in a normal acid dye bath containing about 4 per cent of sulfuric acid, about 5 to 10 per cent of glue, and about 2½ per cent of ammonium fluoride, calculated on the weight of the material to be dyed.

6. The process of dyeing wool with a chromium complex compound of an organic acid dyestuff which comprises carrying out the dyeing in a normal acid dye bath containing about 4 per cent of sulfuric acid, about 2 to 3 per cent of the condensation product from 20 mols ethylenoxyde and 1 mol. octodecylalcohol and about 2½ per cent of ammonium chloride, calculated on the weight of the material to be dyed. 5

7. The process of dyeing wool with a chromium complex compound of an organic acid dyestuff which comprises carrying out the dyeing in a normal acid dye bath containing about 4 per cent of formic acid and about 2 to 3 per cent of a condensation product from ethylenoxyde and do-decylalcohol, calculated on the weight of the material to be dyed. 13

8. The process of dyeing animal fibers with a metal complex compound of an organic acid dyestuff which comprises carrying out the dyeing in a normal acid dye bath containing about 3 to 5 per cent of sulfuric acid and about 2 to 10 per cent, calculated on the weight of the material to be dyed, of the condensation product from an alkylene oxide and a high molecular weight 25 aliphatic alcohol.

9. A dye bath for dyeing animal fibers with metal complex compounds of organic acid dyestuffs comprising a metal complex compound of an organic acid dyestuff, about 3 to 5 per cent 30 of acid as is usual for dyeing with ordinary acid dyestuffs and a water soluble protective colloid.

CARL MARIA RITTINGHAUSEN.  
RICHARD HAYNN.